

April 21, 1942.

W. B. CAMPBELL ET AL

2,280,216

METHOD OF IMPREGNATING FIBROUS MATERIALS

Filed May 5, 1939



INVENTORS  
WILLIAM BOYD CAMPBELL  
OTTO MAASS  
ERNEST EDWARD MASSEY

BY *J. D. O'Connell*  
ATTORNEY

## UNITED STATES PATENT OFFICE

2,280,216

## METHOD OF IMPREGNATING FIBROUS MATERIALS

William Boyd Campbell, Montreal, Quebec, Otto Maass, Westmount, Quebec, and Ernest Edward Massey, Montreal, Quebec, Canada, assignors to Imperial Tobacco Company of Canada, Limited, Montreal, Quebec, Canada

Application May 5, 1939, Serial No. 271,950

4 Claims. (Cl. 91—70)

This invention relates to a method and apparatus for impregnating paper or other material, in the form of rolls or stacks, with wax or other organic or inorganic solids capable of being dissolved in a solvent that will not adversely affect the rolled or stacked material.

The principal object is to enable the wax or other impregnation of paper or other material, in the form of rolls or stacks, to be effected under conditions favorable to the uniform application of the impregnating material and to the maximum recovery of the solvent or solvents contained in the treating solution.

In treating rolls or stacks of paper in accordance with this invention it is important that the wax or other solids to be incorporated in or applied to the paper should be dissolved in solvents that will not cause the paper to swell or deteriorate. This is particularly important when the invention is applied, as hereinafter described, to the production of wax impregnated cigarette papers.

Other objects and advantages will be apparent from the following detail description taken in connection with the accompanying drawing, in which the single figure is a diagrammatic illustration of one form of apparatus which may be used in carrying the invention into effect.

Referring more particularly to the drawing 5 designates a vacuum tank in which paper or other fibrous material is treated in accordance with this invention. The treating solution is preferably prepared in the solution tank 6 by introducing the necessary ingredients through valve 7. Alternately, the treating solution may be prepared in a separate mixing vessel and then introduced into tank 6 through said valve. When the apparatus is in use the treating solution is passed from tank 6 to tank 5 and vice versa through line 8 and valve 9. The upper portion of tank 5 is connected, through line 12 to one end of a coil 13 arranged in a tank 14. The remaining end of coil 13 is connected, through line 15, to a vacuum pump (not shown). Line 15 is provided with valves 16 and 17. Line 15 is also provided, at opposite sides of valve 17, with branches 18 and 19 leading to a solvent tank 20. Branches 18 and 19 are provided, respectively, with valves 21 and 22. Lines 12 and 15 are also connected through bypass line 12a 50 equipped with a valve 12b. Line 12 is equipped with valves 12c and 12d, the former being located between the bypass connection 12a and the coil 13 and the latter being located adjacent tank 5.

In putting the apparatus into operation the tank 5 is loaded with the material to be treated and the treating solution is prepared in or introduced into tank 6. At this time valves 7, 16, 17, 12c and 12d are open but valves 21, 22 and 9 are closed. Tank 5 is thus placed under vacuum to establish a desired absolute pressure therein. Valves 16, 12c and 12d are now closed and valve 9 is opened. Since tank 6 is under atmospheric pressure (the valve 7 being still open) the solution contained therein is forced into vacuum tank 5 through line 8 and valve 9. When this transfer is completed valve 9 is closed and the fibrous material in tank 5 is allowed to soak in the treating solution for a suitable period. During this soaking period tank 5 is gradually heated, by heating coil 29, to a temperature above the boiling point of the solvent contained in the treating solution. Owing to resulting vaporization of the solvent contained in the treating solution the pressure in tank 5 becomes greater than that in tank 6 which is at atmospheric pressure. After the fibrous material has thus been soaked in tank 5 for the desired period, valve 9 is opened. Owing to the difference in pressure in the two tanks the treating solution is now returned to tank 6 through line 8 and valve 9. When this transfer of the solution from tank 5 to tank 6 is completed the valve 9 is again closed.

The next step is to evaporate and reclaim the solvent from the impregnated material. To this end a vacuum is drawn on tank 20, coil 13 and line 12 by opening valves 16, 17, 21, 22 and 12c while valves 12b and 12d are closed. When the desired vacuum conditions are thus established in tank 20, coil 13 and line 12, valves 16 and 17 are closed and valve 12d is opened. At this time water from a cooling tower or other source is circulated through the condensing tank 14 by opening valve 25 in the water supply line 26 and valve 27 in the drain line 28. With this particular setting of the valves (valves 16, 17 and 12b being closed and valves 21, 22, 12c and 12d being open) the solvent evaporated from the material in tank 5 is drawn into the solvent tank through valves 12d, line 12, valve 12c, condensing coil 13, line 19 and valve 22. The last traces of solvent are then removed from tank 5 by closing valve 12c and opening valve 12b in pipe bypass line 12a.

The entire procedure described in the foregoing is repeated one or more times before the material under treatment is removed from tank 5. We find that this repetition of treatment is usually necessary to obtain the best results.

During both the impregnation and solvent re-

covery periods tank 8 is heated by passing steam through the previously mentioned heating coil 29 which is contained in a water jacket 30 surrounding the treatment chamber 8a. Tank 5 may also be provided with a central hollow tubular member 31 rising from the bottom of the tank and communicating with the water jacket 30. This member 31 extends upwardly at the centre of the fibrous material being treated and provides additional surface to assist in effecting uniform distribution of the heat derived from coil 29. Tank 8 is also preferably provided with a water jacket 32 containing a heating coil 33 through which steam or other heating agents is passed.

The heating of tanks 5 and 8 may be automatically regulated with the aid of suitable thermostats 34 and 35. These thermostats are arranged in the lower portions of the tank and may be connected in any suitable manner to indicate and/or regulate the steam heating of the tanks.

In one instance in which the invention was used for the production of wax impregnated cigarette paper the treating solution was composed of the following ingredients mixed together in the following proportions, by weight:

|                      | Pounds |
|----------------------|--------|
| Carbon tetrachloride | 150    |
| Beeswax              | 2      |
| Carnauba wax         | 1½     |

In preparing this solution the waxes were melted and poured into the solvent which has previously been heated to 45 to 50° C. The mixture was then stirred to ensure complete solution. When any appreciable interval of time is permitted to elapse between the preparation and use of the solution it is usually necessary to reheat the solution to 45° C. since some wax may separate from the solution during such interval.

While we have described what is now considered to be a preferred embodiment of this invention it will be understood that various modifications may be resorted to in practice. For example, the various control valves may be operated either manually or automatically, and through the agency of any desired operating mechanism.

Having thus described our invention, what we claim is:

1. The herein described method of impregnating fibrous material in the form of rolls or stacks with a treating solution comprising solids dissolved in a volatile solvent which comprises (1) placing said material in a vacuum tank, (2) introducing the treating solution into said tank, (3) permitting said material to soak in the treating solution for a predetermined period during which the tank is gradually heated to a temperature above the boiling point of the solvent contained in the treating solution, (4) withdrawing residual treating solution from the tank at the end of the soaking period and (5) withdrawing the evaporated solvent from said tank while continuing the heating of the latter to evaporate the solvent absorbed by the material

and then repeating steps (2) to (5) inclusive before removing the material from the treating tank.

2. The method of impregnating rolls or stacks of paper with a treating solution consisting of solids dissolved in a volatile solvent which comprises the following steps: (1) introducing the treating solution into a storage tank which is always under atmospheric pressure; (2) placing the rolls or stacks in a treating chamber; (3) placing the treating chamber in communication with a source of suction and then disrupting said communication when a predetermined sub-atmospheric pressure is established in said chamber; (4) placing the evacuated treating chamber in communication with the storage chamber whereby the treating solution is transferred from the storage chamber to the treating chamber by atmospheric pressure; (5) disrupting the communication between said chambers when the transfer of the treating solution is completed; (6) permitting the rolls or stacks to soak in the treating solution for a suitable period while heating the treating chamber to a temperature above the boiling point of the solvent contained in the treating solution; (7) re-establishing communication between the treating chamber and the storage chamber whereby the unabsorbed treating solution is forced back to the storage chamber by the pressure of the evaporated solvent contained in the treating chamber; (8) disrupting communication between said chambers when the transfer of the treating solution from the treating chamber to the storage chamber is completed; (9) removing all solvent from the treating chamber and from the treated material by exhausting the evaporated solvent from said chamber while simultaneously heating said chamber to a temperature above the boiling point of the solvent, and (10) repeating steps 4 to 9 inclusive before removing the material from the treating chamber.

3. The method of impregnating rolls or stacks of paper with a treating solution consisting of solids dissolved in a volatile solvent which comprises subjecting the rolls or stacks to successive soakings in said solution with intermediate removal of the solvent from the paper by the application of heat and suction, the soakings being carried out at a temperature above the boiling point of the solvent contained in said solution.

4. The method of impregnating paper in the form of rolls with a treating solution consisting of waxes dissolved in the carbon tetrachloride which comprises subjecting the rolls to successive soakings in said solution with intermediate removal of the solvent from the paper by the application of heat and suction, the soakings being carried out at a temperature above the boiling point of the solvent contained in said solution.

W. BOYD CAMPBELL.  
OTTO MAASS.  
E. EDWARD MASSEY.